

C. T. CLARK,  
PROCESS FOR WOOD DISTILLATION,  
APPLICATION FILED AUG. 11, 1917.

1,337,342.

Patented Apr. 20, 1920.

Fig. 3.

Fig. 4.



Fig. 1.



Fig. 2.

Charles T. Clark.  
his Attorneys  
Prindle, Wright & Dunlap.

# UNITED STATES PATENT OFFICE.

CHARLES T. CLARK, OF BAY CITY, MICHIGAN, ASSIGNOR TO E. I. DU PONT DE NEMOURS AND COMPANY, OF WILMINGTON, DELAWARE, A CORPORATION OF DELAWARE.

## PROCESS FOR WOOD DISTILLATION.

1,337,342.

Specification of Letters Patent. Patented Apr. 20, 1920.

Application filed August 11, 1917. Serial No. 185,656.

*To all whom it may concern:*

Be it known that I, CHARLES T. CLARK, of Bay City, in the county of Bay, and in the State of Michigan, have invented a certain new and useful Improvement in Processes for Wood Distillation, and do hereby declare that the following is a full, clear, and exact description thereof.

My invention relates to a process for use in wood distillation so as to obtain therefrom charcoal and the usual products of destructive distillation of wood.

The object of my invention is to provide a process by means of which wood may be distilled in a more advantageous manner. More particularly the object of my invention is to provide a wood distillation process in which green wood may be treated without requiring previous drying thereof in the atmosphere, in which the products of the destructive distillation may be obtained much more quickly than hitherto, in which a larger yield is obtained than hitherto, in which a smaller quantity of fuel is needed for heating purposes, in which the cost is decreased due to the small stock of wood required, and in which charcoal of very uniform quality is obtained which is particularly adapted for use in the chemical arts. Further objects of my invention will appear from the detailed description thereof contained hereinafter.

While my process may be carried out in many different ways and while many different forms of apparatus may be used in connection with my invention I have shown only one type of apparatus in the accompanying drawings in which—

Figure 1 is a plan view of an apparatus made in accordance with my invention;

Fig. 2 is a side elevation of the same; and

Figs. 3 and 4 are respectively an elevation and a plan view of one of the wooden blocks such as are treated in accordance with my invention.

In the drawings I have shown two sets of railway tracks 1 and 2 entering a drying chamber 3 having two separate compartments 4 and 5 for receiving the railway tracks 1 and 2 respectively. Partitions 6 and 7 are provided in the chamber 3 to form the two compartments 4 and 5. Inlet doors 8 and 9 are provided to close the inlet ends of the compartments 4 and 5. A chimney 10 is provided at the inlet end to convey

away the moisture and gases from the compartments 4 and 5. Each of the compartments 4 and 5 is adapted to receive three charges of wood each of said charges being comprised of four cars, said wood being cut in the form of short cylinders or plaques 11, substantially three inches long as shown in Fig. 3. Beneath the chamber 3 there is a hot air supply pipe 12 having a plurality of branch pipes 13 one of which is provided for each charge of wood contained in the compartments 4 and 5. Said pipe 12 is connected at its forward end to a pipe 14 leading from a blower 15 and said blower 15 is connected by a pipe 16 to a stack 17 leading from a furnace 17<sup>a</sup> provided for heating a retort 18 in which the wood is to be destructively distilled. In the stack 17 there is a damper 18<sup>a</sup>. Furthermore in the side of the pipe 16 there is a damper 20 to control an inlet port for cold air. The blower 15 is driven by a belt 21 from a shaft 22 which is driven by an engine 23. Said shaft 22 is furthermore connected by a belt 24 to another blower 25 which is adapted to circulate the air in the chamber 3. At the forward end of the chamber 3 there are two doors 26 and 27 through which when open the car loads of wood are adapted to be moved into a connecting chamber 28 leading to a retort house 29 through doors 29<sup>a</sup> and thence into the retort 18 through doors 29<sup>b</sup>. In the connecting chamber there are side doors 30 and 31 to give access thereto. On the retort 18 there is provided any suitable outlet pipe 32 and condenser 33. At the forward end of the retort 18 there are outlet doors 34 and 35 and at the same end of the retort house 29 there are outlet doors 36 and 37.

In the operation of my invention blocks of green hard wood such as maple, birch, beech, oak, etc., are obtained by merely cutting the logs crosswise at intervals of three inches, thus obtaining blocks or plaques of the shape shown in Figs. 3 and 4. These blocks are loaded on cars which are fed into the preliminary heating chamber 3 until said chamber contains three charges of four cars each, that is to say one charge for each of the pipes 13. The doors 8, 9, 26 and 27 of said chamber are now closed and heated air together with the products of combustion from the pipes 13 are supplied beneath the cars of wood so that said air passes

95

90

100

105

110

through and around the piles of blocks contained on the respective cars. The air and products of combustion passing up the stack 17 have such a high temperature that if conveyed unchanged to the wood in the chamber 3 they would ignite the wood, but by supplying cold air by means of the damper 20 the temperature is reduced to 150° C. to 180° C., thus providing a temperature which 10 is entirely safe to be used in heating the wood. The wood in the chamber 3 thus becomes effectively heated by the heat necessarily formed in connection with the distilling operation and furthermore the wood 15 becomes uniformly dried, inasmuch as the moisture driven off by the heat passes out by means of the chimney 10. This dried and hot wood is now fed forwardly by moving the first two charges of four cars 20 each through the intermediate chamber 28 and into the retort 18. Immediately afterward additional charges are introduced at the rear end of the chamber 3 to replace those that have been withdrawn from the 25 forward end thereof, the remaining cars previously present in the chamber 3 having been moved forwardly for this purpose. The distilling operation is now carried on until the wood is entirely carbonized thus 30 obtaining charcoal of uniform quality and the usual distillates obtained in destructive distillation of wood, as for example methyl alcohol, acetic acid, acetone, etc., as well as tar. The cars of charcoal thus 35 obtained are now removed from the retort 18 through the doors 34, 35, 36 and 37 and additional cars are moved forward to take their places in a similar manner. The total period of time required from the beginning 40 of the heating operation to the end of the distillation in accordance with my invention is usually twenty-four hours. In this way the process is a continuous one, inasmuch as that as soon as the treatment of a 45 part of the wood has been completed other partially treated wood is moved up to take its place and other untreated wood is also introduced at the same time.

In accordance with my process, therefore, 50 it is not necessary to allow the wood to dry for months at a time, as was formerly the case, prior to the distilling operation but the wood while in its green state may be treated at once so that the entire operation 55 from the green wood to the completed charcoal requires only twenty four hours for its treatment. In this way the large expense due to maintaining large stocks of wood on hand during the drying of the same in the 60 atmosphere is avoided. Furthermore, carbonization takes place more rapidly because of the wood having been heated before it is introduced into the still and at a

lower temperature because of the previous heating thereof and also with a lower expenditure of fuel as some of the heat which formerly passed away with the products of combustion at the still is transferred to the wood prior to its introduction into the still. Again, because of the shape of the blocks 65 70 the carbonization takes place more rapidly and uniformly as wood may be carbonized more readily and rapidly by progressive action in the direction of the grain than across the grain. Also higher yields of distillates are obtained by the treatment of the green wood than in the previous treatment of air dried wood as the air drying of the wood usually results in bringing about some decay therein. The charcoal obtained has a 75 80 very uniform quality and is particularly well adapted for use in making powder and for metallurgical purposes.

While I have described my invention above in detail I wish it to be understood 85 that many changes can be made therein without departing from the spirit of my invention.

What I claim is:

1. The process of wood distillation which 90 comprises preheating wood which has been cut transversely to the grain into plaques whose dimension parallel to the grain is less than a dimension perpendicular to the grain, and then introducing the heated wood 95 into a retort and subjecting it to destructive distillation.

2. The process of accelerating the distillation of wood which comprises cutting green wood transversely to the grain into 100 short cylinders, preheating the cylinders to dry them and then subjecting the preheated cylinders to destructive distillation.

3. The process of accelerating the distillation of wood which comprises cutting 105 the wood transversely to the grain into plaques about three inches in length, and subjecting the plaques with their surfaces exposed to the atmosphere of the retort to a high temperature sufficient to cause destructive distillation thereof.

4. The process of accelerating the distillation of wood which comprises cutting the wood transversely to the grain into 110 plaques about three inches in length, and subjecting the plaques with their surfaces exposed to the atmosphere of the retort to a high temperature sufficient to cause destructive distillation thereof, said wood being preheated by the heat from the retort.

In testimony that I claim the foregoing I have hereunto set my hand.

CHARLES T. CLARK.

Witnesses:

BEN E. SHORE,  
JAMES R. OWEN.